

## UNITED STATES PATENT OFFICE

2,316,347

## STEAM CYLINDER OIL

Frederick H. MacLaren, Calumet City, Ill., assignor to Standard Oil Company, Chicago, Ill., a corporation of Indiana

No Drawing. Application June 27, 1940,  
Serial No. 342,683

14 Claims. (Cl. 252—56)

This invention relates to lubricants for valves or other mechanical parts that are exposed to steam, such as steam cylinder oils and the like.

The object of the present invention is to provide a lubricant which will withstand severe operating conditions, which will maintain a continuous resistant lubricating film on and between the metal surfaces to be lubricated and which will provide superior lubrication with minimum oil consumption. A further object is to provide a lubricant which will increase the efficiency of steam engines or compressors in which it is used. A further object is to provide a lubricant of the type described which is stable and which is unlikely to decompose and separate out. Other objects and advantages of the present invention will become apparent as the detailed description of the invention proceeds.

My improved steam cylinder oil comprises a blend of about 55% to about 81.8% of a heavy lubricating oil such as for example heavy steam refined oil, from about 3% to about 14% of a fatty material such as lard oil, tallow oil, hydrogenated fat or similar material from about 0.2% to about 1% of a component capable of reducing the drop size of the lubricant such as sperm oil, aluminum stearate or lead soaps, for instance lead oleate, lead fish oil soap or the like, and from about 15% to about 30% of a synthetic lubricating oil of the type hereinafter described.

The synthetic oil is obtained by the polymerization of isomono-olefins such as isobutylene or hydrocarbon mixtures containing the same in the presence of a catalyst such as boron fluoride, aluminum chloride, zinc chloride or other similar active halide catalyst adapted to promote the Friedel-Crafts synthesis, at a temperature of from about 0° F. to about 100° F. Co-polymers formed by the polymerization of mixtures of olefins, preferably of an iso-olefin such as isobutylene with other olefins of the same or a different number of carbon atoms per molecule, are also suitable for this purpose. In the preparation of this synthetic oil I may employ liquid isobutylene or a hydrocarbon mixture containing the same, such as for example a butane-butylene fraction recovered from petroleum gases, especially those gases produced in the cracking of petroleum oils for the manufacture of motor fuels. This light fraction may contain from about 10% to about 25% isobutylene, the remainder being principally butanes and normal butylene.

The synthetic oil may be prepared, for example, by maintaining the liquid isobutylene or the hydrocarbon mixture containing the same under pressure and cooling the same to a temperature for example of about 32° F. and introducing from about 0.1% to about 2% of boron fluoride with vigorous agitation. Excessive rise

in temperature due to the heat of reaction may be avoided by efficient cooling. To facilitate agitation of the mixture and to control the reaction temperature I prefer to employ a light diluent such as hexane, liquid butane, liquid propane and the like. By effecting the evaporation of the light diluent efficient cooling and control of the reaction temperature is obtained. After polymerization of the isobutylene the reaction mass is neutralized, the oily polymer layer separated from the sludge and the polymers subsequently separated from the unreacted light hydrocarbons by distillation.

The synthetic polymer obtained as above described is subsequently fractionated by first introducing the same into a flash tower maintained at the lowest pressure commercially feasible, for example from about 1 to about 6 inches of mercury, and at a temperature of from about 400° F. to about 600° F. wherein the polymer is flash distilled and the vapors removed overhead for subsequent fractionation. The unvaporized portion in the flash tower which is the material I prefer to use, and refer to herein as "flasher bottoms", is withdrawn from the flash tower. The flasher bottoms have a Saybolt Universal viscosity at 210° F. of from about 1500 seconds to about 4000 seconds, an A. P. I. gravity of from about 23° to about 26°, a flash of from about 510° F. to about 570° F. and a molecular weight of from about 1000 to about 1500.

Having described the constituents of my improved valve oil the following formulae will exemplify a preferred embodiment of the invention:

## Example

|                                                                                                                                                                                                                                                                                                                                                                                                                                                                                                                                                                                                                                                                                        | Preferred | Preferred range |
|----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-----------|-----------------|
| 40                                                                                                                                                                                                                                                                                                                                                                                                                                                                                                                                                                                                                                                                                     |           |                 |
| Sperm oil                                                                                                                                                                                                                                                                                                                                                                                                                                                                                                                                                                                                                                                                              | 0.5       | 0.2-1.0         |
| Prime lard oil                                                                                                                                                                                                                                                                                                                                                                                                                                                                                                                                                                                                                                                                         | 5         | 3.0-14.0        |
| Steam refined oil                                                                                                                                                                                                                                                                                                                                                                                                                                                                                                                                                                                                                                                                      | 74.5      | 55.0-81.8       |
| Flasher bottoms                                                                                                                                                                                                                                                                                                                                                                                                                                                                                                                                                                                                                                                                        | 20        | 15.0-30.0       |
| 45                                                                                                                                                                                                                                                                                                                                                                                                                                                                                                                                                                                                                                                                                     |           |                 |
| In the above formula the steam refined oil may be a heavy steam refined Mid-Continent lubricating oil having a flash point of about 530° F. and a Saybolt Universal viscosity at 210° F. of about 175 to about 200 seconds. Instead of using a Mid-Continent steam refined oil I may use a heavy Pennsylvania steam refined oil or a heavy steam refined oil from Wyoming crude oils, or I may use mixtures of these heavy steam refined oils. For example, a suitable blend is one comprising about 47% of a heavy steam refined oil from Wyoming crude and about 27½% of a heavy Pennsylvania steam refined oil having a Saybolt Universal viscosity of about 185 seconds at 210° F. |           |                 |

50

55

60

The inspection of the valve oil exemplified by the above preferred formula is as follows:

|                                        |          |      |
|----------------------------------------|----------|------|
| Flash                                  | °F.      | 580  |
| Pour                                   | °F.      | +25  |
| Saybolt Universal viscosity at 210° F. | seconds  | 257  |
| Drop size                              |          | .08  |
| Tarry matter                           | per cent | .008 |

In the lubrication of compressors, steam engines and similar apparatus it is the common practice to supply the oil through a dropper or a hydrostatic lubricator, and it is therefore of extreme importance that the drop size be uniform and constant. Valve oils having the composition herein described have a drop size which is uniform and constant and of such size to provide the maximum effective lubrication with a minimum consumption of oil.

While I have described in detail a preferred embodiment of my invention, it is to be understood that I do not wish to limit myself to the specific materials and proportions above-stated except as defined by the following claims.

I claim:

1. A cylinder oil comprising a major proportion of a heavy lubricating oil, small amounts of a fatty oil, and a drop size reducing agent, and at least about 15% of an isobutylene polymer having a molecular weight within the range of from about 1,000 to 1,500.

2. A cylinder oil comprising about 55% to about 81.8% heavy steam refined lubricating oil, about 3% to about 14% fatty material, about 0.2% to 1.0% of a drop size reducing agent, and about 15% to 30% isobutylene polymer having a molecular weight within the range of from about 1,000 to about 1,500.

3. A cylinder oil comprising the following approximate composition by weight percentage:

|                                           | Per cent  |
|-------------------------------------------|-----------|
| Sperm oil                                 | 0.2-1.0   |
| Prime lard oil                            | 3.0-14.0  |
| Steam refined oil                         | 55.0-81.8 |
| Iso-mono-olefin polymer "flasher bottoms" | 15.0-30.0 |

4. A cylinder oil comprising the following in-

gredients in the approximate proportions by weight percentage:

|                                           | Per cent |
|-------------------------------------------|----------|
| Sperm oil                                 | 0.5      |
| Lard oil                                  | 5.0      |
| Steam refined oil                         | 74.5     |
| Iso-mono-olefin polymer "flasher bottoms" | 20.0     |

5. A cylinder oil as described in claim 4 in which the drop-size reducing agent is sperm oil.

6. A cylinder oil as described in claim 4 in which the drop-size reducing agent is aluminum stearate.

7. A cylinder oil as described in claim 4 in which the drop-size reducing agent is lead soap.

8. A cylinder oil comprising about 55% to about 81.8% heavy lubricating oil, about 3% to about 14% fatty material, about 0.2% to about 1% of a drop-size reducing agent and about 15% to about 30% of an iso-mono-olefin polymer having a molecular weight within the range of from about 1,000 to about 1,500.

9. A cylinder oil as described in claim 8 in which the drop-size reducing agent is sperm oil.

10. A cylinder oil as described in claim 8 in which the drop-size reducing agent is aluminum stearate.

11. A cylinder oil as described in claim 8 in which the drop-size reducing agent is a lead soap.

12. A cylinder oil comprising about 55% to about 81.8% heavy lubricating oil, about 3% to about 14% fatty material, about 0.2% to about 1% of a drop-size reducing agent and about 15% to about 30% of an iso-mono-olefin polymer having a Saybolt Universal viscosity at 210° F. of from about 1,500 seconds to about 4,000 seconds.

13. A cylinder oil comprising a major proportion of a heavy lubricating oil, small amounts of a fatty oil, and a drop-size reducing agent and at least about 15% of an iso-mono-olefin polymer having a Saybolt Universal viscosity at 210° F. of from about 1,500 seconds to about 4,000 seconds.

14. A cylinder oil comprising a major proportion of a heavy lubricating oil, small amounts of a fatty oil, and a drop-size reducing agent and at least about 15% of an iso-mono-olefin polymer having a molecular weight within the range of from about 1,000 to about 1,500.

FREDERICK H. MACLAREN.

CERTIFICATE OF CORRECTION.

Patent No. 2,316,347.

April 13, 1943.

FREDERICK H. MacLAREN.

It is hereby certified that error appears in the printed specification of the above numbered patent requiring correction as follows: Page 2, second column, lines 9, 11 and 14, for "claim 4" read --claim 2--; and that the said Letters Patent should be read with this correction therein that the same may conform to the record of the case in the Patent Office.

Signed and sealed this 1st day of June, A. D. 1943.

Henry Van Arsdale,  
Acting Commissioner of Patents.

(Seal)